

W. SCHEMANN & J. BRONN.  
PROCESS OF MELTING FERRO ALLOYS AND KEEPING THEM IN LIQUID STATE.  
APPLICATION FILED DEC. 30, 1912.

1,061,016.

Patented May 6, 1913.



Fig. 1.



Fig. 2.



Fig. 6.



Fig. 7.



Fig. 3.



Fig. 4.



Fig. 5.

Witnesses:  
John Murtagh  
Grace Lane

5

Wilhelms Schermann Inventor  
By his Attorney, George R. Tracy  
G. R. Tracy

# UNITED STATES PATENT OFFICE.

WILHELM SCHEMMANN AND JEGOR BRONN, OF ROMBACH, GERMANY, ASSIGNEES TO ROMBACHER, HÜTTENWERKE, OF ROMBACH, GERMANY, A CORPORATION OF GERMANY.

## PROCESS OF MELTING FERRO-ALLOYS AND KEEPING THEM IN LIQUID STATE.

1,061,016.

Specification of Letters Patent.

Patented May 6, 1913.

Application filed December 30, 1912. Serial No. 739,288.

To all whom it may concern:

Be it known that we, WILHELM SCHEMMANN and JEGOR BRONN, citizens of the German Empire, residing at Rombach, in said German Empire, have invented certain new and useful Improvements in Processes of Melting Ferro-Alloys and Keeping Them in Liquid State, of which the following is a specification.

10 The advantages of an addition of ferro-manganese in liquid form to the ingot-iron or mild steel to be deoxidized, have been pointed out heretofore by us in United States Letters Patent No. 915,488 obtained by us, and we have recommended for this purpose the employment of an electric furnace with pure resistance heating. It has been found, however, by continuous practical working of these furnaces that although 20 metal could be easily melted in the trough-furnaces therein suggested, that gradually a great deal of slag was collected in the melting trough, which slag remained tough and had to be removed from time to time by 25 means of tools, which caused frequent interruptions in the working of the furnaces, while the troughs were liable to be subjected to damage. When, however, it is attempted to melt ferro-manganese in an electric arc-furnace such as is generally used for refining steel, a thick brown smoke begins at once to escape from the furnace owing to the combustion and evaporation of the manganese, and the loss of manganese which takes place 30 is so great that the remelting of ferro-manganese becomes unprofitable.

It is well known that in electric arc-furnaces which are used in the refining of steel, the drop of the tension within the electric 40 arc, that is to say, when measured between the carbon-block and the metal bath, amounts to from 45-75 volts. It has been found, however, that when the carbon electrode is lowered to such an extent that it 45 just touches the surface of the bath, and that when such a tension of the current is used, that the difference or drop of tension between the carbon and the metal bath amounts to only from 16-18 volts, and that 50 this drop is below the electromotive counter-force of the arc, which is generally taken to be about 30 volts, it is possible to obtain, by the contact-resistance thus produced, an

amply sufficient heating of the melting bath without any noticeable loss of manganese 55 taking place.

In view of the fact that in carrying out the present invention, the electrode just touches the free surface of the metal bath, the heating cannot be regarded as being effected by means of an ordinary flame arc, but by means of the contact resistance between the electrode and the free surface of the bath. The term "contact resistance heating" is therefore used hereafter to distinguish this method of heating from the ordinary flame arc and from ordinary resistance heating, and is in fact, similar to the known method of heating by bad surface contact or so-called "semi-arching" which 70 method has been used for melting ferro-manganese.

The invention consists in a process for melting ferro-manganese and similar alloys in which the melting is effected by means of 75 contact resistance heating, the voltage drop between each of the movable block electrodes and the bath of molten material being less than thirty volts.

The accompanying drawings illustrate by 80 way of example some constructions of a furnace for carrying out this invention.

Figures 1 and 2, are vertical cross sections at right angles to each other of a furnace for three phase current. Figs. 3 and 4 are 85 respectively, a sectional plan and a sectional elevation of a modified construction of furnace. Fig. 5 is a sectional plan of a modification of the preceding construction. Figs. 6 and 7 are respectively a sectional 90 elevation and a plan of a further modification.

The furnace shown in Figs. 1 and 2 is designed for three-phase current; it is similar in its construction to the usual steel furnaces and like these it can also be operated with ordinary alternating current, that is to say with only two electrodes. It is however indispensable that, as already stated, the voltage drop between each electrode and the 95 bath shall not exceed the limits above stated. This can be easily effected by arranging that the source of current to which the electrodes are to be connected shall supply a current of suitable low voltage. In most cases the 100 current can be supplied by stationary trans-

formers. When for instance, a single phase electric furnace having only one contact resistance between the movable electrode and the metal bath (Figs. 6 and 7) is required to work in the manner herein described with a voltage drop of about 20 volts, then the voltage between the secondary terminals of the transformer must not exceed 20 volts (including any loss of voltage). In single phase furnaces having two movable electrodes, the voltage drop between each electrode and the metal bath must amount to 20 volts. This discovery that by a kind of heating by contact resistance it is possible to obtain a supply of heat which is quite sufficient for melting and keeping in the molten state ferro-manganese and the resulting slag, may be applied directly to a furnace of the type illustrated in Figs. 3 and 4. The metal bath is inserted as a heating resistance in a channel, and the slag which forms on the surface of the bath and which is not sufficiently heated by the resistance heating, is, however, kept hot by the heat developed owing to the contact resistance between the free surface of the metal bath and the electrodes. The slag above referred to is formed owing to the fact that, during the heating a layer of oxids forms on the surface of the metal which oxids attack the material of the furnace and thus form slag. It is to be understood that only a very thin layer of slag is formed which is blown back or forced away around the electrode by the action of the electric current. In working this combined furnace with three-phase current, as shown in Figs. 3 and 4, has the following advantages over the furnace shown in Figs. 1 and 2 namely: 1. The consumption of the expensive movable block electrodes is reduced to one third, and the labor of changing and adjusting the electrodes is diminished. 2. The actual bath and the covering layer of slag can be heated independently of each other at will with much greater convenience because the metal bath is heating chiefly in the channels by pure resistance heating whereas the slag covering on the bath is heated by means of the contact resistance as described above. This regulation of the heating is effected most simply by keeping the level of the bath in the channels higher or lower whereby the conductive cross sectional area of the metal bath, and consequently also the current passing through the same is varied. The cross section of the channels 1 and 2 is preferably made such that the internal resistance of the metal bath in them is approximately equal to the resistance between the metal bath and the electrode 9. As shown in Figs. 3 and 4 the two channels 1 and 2 open into a wide hearth 3 which is heated by means of the electrode 9. Blocks 4 of carbon or

graphite are arranged at the two closed ends of the channels. We have discovered that unlike ingot iron ferro-manganese is not capable of dissolving carbon. Consequently the electrode blocks 4, which are let into the ends of the channels are practically not subjected to any wear and tear except where they come in contact with the external atmosphere, that is to say, at their upper parts where they are raised to incandescence by the heat of the current and the heat of conduction, so that a slow combustion takes place. With the object of reducing this wear and tear as far as possible and of avoiding the inconvenient unmaking and remaking of the contacts or connections for the heavy current supply the current connections are arranged as follows:—Flexible cables lead from the terminals of the transformers to the copper bars 5. These copper bars are clamped around a water cooled metal body 6 mounted on carbon slabs resting on the carbon block 4. For the purpose of maintaining a very intimate contact between the metal body and the block 4, the metal body 6 is pressed against the block by means of a steel screw 7 and an intermediate insulating piece 8. The two channels 1 and 2, and the carbon or graphite block 9 which depends into the hearth, are connected respectively to the current phases *a* *b* *c* of the three phase current. Fig. 5 is a cross section of a similar furnace which is however, worked with single-phase alternating current.

In working the furnace constructed as shown in Figs. 3 and 4, it is advisable to charge the furnace with ferro-manganese in small lumps. If the ferro-manganese is charged mainly in large lumps into the furnace these lumps melt but slowly and thus interfere with the continuous working which ought to keep step with the working of the steel making plant. For this reason it may be preferable under certain circumstances to employ, instead of the furnace shown in Figs. 3 and 4, a series of furnaces as shown in Figs. 6 and 7 for working in connection with steel-making plant. Each of the three furnaces can be connected according to the available voltage, either to two phases of the three-phase current, for instance:—furnace I to the phases *a* and *b*, furnace II to the phases *b* and *c*, furnace III to the phases *a* and *c*, or if the voltage is too high it may be connected to the two terminals belonging to the same phase. These three furnaces work simultaneously, except that they are charged and discharged intermittently. Since never more than four converter charges per hour are made even in the largest steel works, each furnace has therefore three quarters of an hour for heating and melting the fresh charge of ferro manganese.

The furnaces hereinbefore described are

very suitable for melting other readily combustible or vaporizable ferro alloys especially when these are rich in carbon.

Having now particularly described and ascertained the nature of our said invention and in what manner the same is to be performed, we declare that what we claim is:—

1. The process herein described of melting ferro-manganese and similar alloys which consists in melting the alloys by means of contact resistance heating using a voltage drop between each of the movable block electrodes and the bath of molten material which is less than thirty volts.
- 15 2. The process herein described of melting ferro-manganese and similar alloys which consists in melting the alloys by means of contact resistance heating in conjunction with ordinary resistance heating

using a voltage drop between each of the 20 movable block electrodes and the bath of molten material which is less than thirty volts.

3. The process herein described of melting ferro-manganese and similar alloys which 25 consists in so disposing the movable electrode that the drop or difference of tension between the electrodes and the bath is less than 30 volts.

In testimony, that we claim the foregoing 30 as our invention, we have signed our names in presence of two subscribing witnesses.

WILHELM SCHEMMANN.  
JEGOR BRONN.

Witnesses:

LOUIS VANDORY,  
BESSIE F. DUNLAP.